

## UNITED STATES PATENT OFFICE

2,645,605

## REFORMING AND CATALYSTS THEREFOR

William H. Lang, Wenonah, and Carlos L. Gutzeit,  
Woodbury, N. J., assignors to Socony-Vacuum  
Oil Company, Incorporated, a corporation of  
New York

No Drawing. Application April 27, 1951,  
Serial No. 223,438

4 Claims. (Cl. 196—50)

1

This invention relates to new reforming catalysts characterized by the combination, in a single catalyst composition, of the catalytic properties of isomerization and of aromatization, and to a process for effecting naphtha reforming utilizing these catalysts. More particularly, the present invention is concerned with new reforming catalysts containing chromia, fluorine and an amphoteric metal.

As is well known to those familiar with the art, unsaturated hydrocarbons, as a class, possess octane number ratings that are higher than those of the corresponding saturated hydrocarbons, and aromatic hydrocarbons, as a class, possess octane number ratings that are higher than those of aliphatic and naphthenic or alicyclic hydrocarbons, saturated and unsaturated, although the octane number ratings of certain aliphatic hydrocarbons are as high or even higher. In general, therefore, the conversion of saturated hydrocarbons into unsaturated hydrocarbons through dehydrogenation, and the conversion of aromatizable aliphatic and alicyclic hydrocarbons into aromatic hydrocarbons through dehydrogenation or cyclization or both, i. e., dehydrocyclization, depending upon the type of aromatizable hydrocarbon, are expedients whereby the low-octane hydrocarbons are converted into the corresponding higher-octane hydrocarbons. The reactions involved are well known and several processes, involving these reactions, have been proposed for the purpose of producing gasolines having improved antiknock properties from petroleum naphthas. These operations are generically referred to as reforming and the conditions of temperature, pressure (including hydrogen pressure), and residence time are referred to as reforming conditions.

Most of the proposed reforming processes involve the use of catalysts. Depending upon the type of reaction or reactions which they primarily promote, the reforming catalysts have been termed aromatization catalysts, dehydrogenation catalysts, dehydrocyclization catalysts, etc. Indeed, these catalysts also promote cracking, thereby producing normally gaseous hydrocarbons and carbonaceous deposits on the catalysts.

Controlled or selective cracking is advantageous from two standpoints. In the first place, it increases the yields of desired product, through the conversion of the higher-boiling constituents of the charge stocks into fractions boiling within the gasoline boiling range (80° F. to 400° F.) and by decreasing the conversion of fractions boiling within the gasoline boiling range into normally

2

gaseous hydrocarbons. In the second place, it further increases the octane number rating of the reformed gasoline through the formation of unsaturated hydrocarbons. Excessive and uncontrolled cracking, on the other hand, although increasing the formation of unsaturated hydrocarbons, increases the amounts of normally gaseous hydrocarbons and of carbonaceous deposits with concomitant losses in the yields of desired product and rapid deactivation of the catalyst. Accordingly, as is well known to those familiar with the art, the performances of reforming catalysts are ordinarily compared on the basis of octane number rating—gasoline yield relationships.

10 Chromia-on-alumina is typical of the reforming catalysts of the prior art. Its function in reforming operations is as a dehydrogenation-dehydrocyclization catalyst. It does not promote isomerization to any great extent and is not selective in its cracking activity. Thus, in a typical reforming operation in which a chromia-on-alumina reforming catalyst is employed, a saturated gasoline, such as, for example, a straight-run gasoline, which comprises a mixture of paraffinic and alicyclic hydrocarbons, is subjected to reforming conditions, whereby, the aromatizable alicyclic hydrocarbons are dehydrogenated into aromatic hydrocarbons and the aromatizable paraffinic hydrocarbons are dehydrocyclized into aromatic hydrocarbons. The improved octane number rating of the reformed gasoline obtained from such an operation may be attributed, therefore, primarily, to the formation of the aromatic hydrocarbons.

15 It is well known that chromia-on-alumina catalysts are among the most active of the dehydrocyclization catalysts. This high activity is obtained at low pressures, such as atmospheric, and at temperatures of the order of 900—1000° F.

20 It is also well known that when dehydrocyclization catalysts, such as chromia-alumina, are employed under hydrogen pressure, the dehydrocyclization activity is preferentially decreased, compared to the dehydrogenation of naphthenes containing six-membered rings. In spite of this, it has become common practice to use such catalysts under hydrogen pressure in order to gain the advantage of reduced coke deposition. Such operations are predicated upon striking a balance between the practical advantages of reduced coke formation and the decreased aromatization, especially the reduced dehydrocyclization, obtained under hydrogen pressure.

25 As stated hereinbefore, the octane number ratings of certain aliphatic hydrocarbons are as

high or even higher than those of aromatic hydrocarbons. These aliphatic hydrocarbons are highly-branched, a structure ordinarily obtained through isomerization of the corresponding, less highly-branched aliphatic hydrocarbons. Accordingly, a reforming catalyst which promotes isomerization reactions is manifestly highly desirable.

In copending application for patent Serial No. 216,460, filed on March 19, 1951, by Rowland C. Hansford, there is disclosed and claimed a catalyst containing chromia, specified amounts of fluorine, and alumina. In accordance with copending application Serial No. 218,291, filed on March 29, 1951, by Carlos L. Gutzeit, these chromia - fluorine - alumina catalysts promote aromatization and isomerization reactions in reforming operations involving hydrogen pressure.

From a theoretical standpoint, the chromia-fluorine-alumina catalysts are capable of producing gasoline in the highest yield for a given octane number rating. This follows from the fact that these catalysts effect the conversion of cyclohexanes and of alkyl cyclopentanes into aromatic hydrocarbons with a smaller increase in density than is the case in the dehydrocyclization of aromatizable paraffinic hydrocarbons and, also, effect the isomerization of paraffinic hydrocarbons with concomitant increase in octane number rating and with substantially no volume change.

In the copending applications referred to, it was found that, in accordance with the teachings of the prior art, in aromatization reforming at atmospheric pressure, the fluorine-containing chromia-alumina catalysts were inferior to the fluorine-free chromia-alumina catalysts. Also, in accordance with the prior art, it was found that, in reforming operations involving the use of fluorine-free chromia-alumina catalysts, hydrogen pressure showed a tendency to suppress aromatization activity, so that it was necessary to increase temperature and/or apparent contact time in order to maintain the conversion by such catalysts at a reasonable level. Such compensatory octane number level with reduced coke formation could be achieved at pressures of up to 200 pounds per square inch gauge and a hydrogen-to-naphtha mole ratio varying between about 2:1 and about 10:1, respectively, with only minor disadvantages in the octane number rating-gasoline yield relationship. However, at pressures of 500 pounds per square inch gauge and higher, using hydrogen dilutions falling within the same range of variation and under conditions of negligible coke formation, the fluorine-free chromia-alumina catalysts were not sufficiently active, in reforming operations, to be commercially feasible.

On the other hand, it was found that, under hydrogen pressure, the addition of small amounts of fluorine to conventional chromia-alumina reforming catalysts improved their activity. Indeed, tests showed that, within reasonable limits, the effectiveness of fluorine in this respect increased as the pressure increased. Thus, for example, the addition of small amounts of fluorine to a chromia-alumina catalyst (mole ratio=Cr<sub>2</sub>O<sub>3</sub>:Al<sub>2</sub>O<sub>3</sub>::24:76), using a hydrogen-to-naphtha mole ratio of 4:1, caused slight inferiority at atmospheric pressure, slight superiority at 200 pounds per square inch gauge, and marked superiority at 500 pounds per square inch gauge. At pressure of 500 pounds per square inch gauge and higher, the coke deposition was negligible,

thereby permitting continuous operation for long periods without interruption for oxidative regeneration to remove carbonaceous material.

In the copending applications, it was stated that the improvement in activity of the fluorine-containing chromia-alumina catalysts under hydrogen pressure was due to a superposition of isomerization activity on the dehydrogenation activity of the chromia-alumina catalysts. Under optimum conditions for dehydrocyclization, such as at atmospheric pressure, this isomerizing action caused only a small part of the octane number rating increase but caused a marked increase in coke formation, resulting in an overall deleterious effect. Under increased hydrogen pressure, where dehydrocyclization was diminished and coke formation became small or negligible, the isomerization contributed a very considerable part of the over-all octane number rating increase, and the over-all activity of the catalyst for aromatization reforming was increased.

Isomerization-aromatization catalysts may be considered to be bifunctional catalysts, one function being that of cracking-isomerization and the other that of dehydrogenation, although these functions need not be entirely separate and distinct. The chromia-fluorine-alumina catalysts belong to the class wherein such functions are distinct and can be separately controlled by a judicious selection of the active components. The fluorine or acid component functions as the cracking-isomerization promoter while the chromia component functions as the dehydrogenation promoter. While the alumina component is not strictly non-catalytic, it may, as a first approximation be considered to be merely an activating support which acts as a high surface-area carrier for the catalytically active material and to prevent crystallization, migration or volatilization of active components. Therefore, the ratio of fluorine to chromia was selected so that the fluorine component would produce isomerization but only negligible cracking, while the chromia component promoted the dehydrogenation of the aromatizable alicyclic hydrocarbons at the relatively high space velocities necessary to effect selective isomerization with the fluorine component.

Accordingly, the reforming catalysts of the copending application filed by Hansford comprise combinations of from about 5 per cent by weight to about 70 per cent by weight of chromia, calculated as Cr<sub>2</sub>O<sub>3</sub>, with from about 0.1 per cent by weight to about 2.0 per cent by weight of fluorine, and the balance, an active alumina base. More particularly preferred, however, are stated to be combinations of from about 10 per cent by weight to about 35 per cent by weight of chromia, calculated as Cr<sub>2</sub>O<sub>3</sub>, with from about 0.2 per cent by weight to about 1.5 per cent by weight of fluorine, and the balance, an active alumina base.

The chromia-fluorine-alumina catalysts of this copending application were found to be unstable under oxidizing conditions, either during catalyst preparation or during oxidative regeneration. Indeed, the specification of the copending application states that it is essential to effect the calcination in a hydrogen atmosphere. For this reason, as set forth in the copending application filed by Gutzeit, the indicated and preferred use of these chromia-fluorine-alumina catalysts is in reforming operations involving relatively high hydrogen pressures, of the order of 500 pounds per square inch gauge and higher. As stated

hereinbefore, at these pressures, the coke deposition is so low as to preclude the necessity of oxidative regeneration of the catalyst, thereby permitting continuous operation for long periods of time. Eventually, of course, the coke deposit will reach such a magnitude as to seriously impair the activity of the catalyst. In normal, commercial operations, and using catalysts that are stable under oxidative conditions of regeneration, the catalysts would be regenerated and reused. If the chromia-fluorine-alumina catalyst is so treated, the fluorine-content of the catalyst is lost rapidly and with it, the advantages of the catalyst. Accordingly, expedients whereby these chromia-fluorine-alumina catalysts are stabilized are manifestly of considerable commercial significance.

It has now been discovered that it is possible to stabilize these chromia-fluorine-alumina reforming catalysts. It has been found that the addition of certain amphoteric metals, viz., antimony, tin and bismuth, in specified amounts, effects the stabilization of the fluorine in chromia-fluorine-alumina reforming catalysts.

The addition of amphoteric metals to chromia-alumina dehydrocyclization catalysts is well known. Thus, for example, antimony has been added to chromia-alumina catalysts as a promoter. The function of the amphoteric metals herein is not that of a promoter, but that of a stabilizer for fluorine.

Accordingly, it is an object of this invention to provide improved reforming catalysts. Another object is to provide efficient aromatization-isomerization catalysts. Still another object is to provide improved chromia-alumina reforming catalysts. A further object is to afford an improved reforming process. An important object is to provide a catalytic reforming process to achieve improved octane number rating-gasoline yield relationships. A more specific object is to provide a catalytic reforming process utilizing a catalyst containing chromia, specified amounts of fluorine, specified amounts of an amphoteric metal, and alumina, and hydrogen pressures. Other objects and advantages of the present invention will become apparent to those skilled in the art from the following description.

Broadly stated, the present invention provides:

1. A reforming catalyst comprising a combination of specified amounts of chromia with specified amounts of fluorine and specified amounts of an amphoteric metal selected from the group consisting of antimony, tin and bismuth, supported on an active alumina base; and

2. A process for effecting reforming of petroleum naphthas, which comprises contacting a petroleum naphtha with the aforesaid reforming catalyst, under reforming conditions including hydrogen partial pressures.

In accordance with the present invention, the amount of antimony, tin or bismuth to be incorporated in the catalyst must be equal to from about 0.5 to about 2 times, preferably, from about 0.5 to about 0.75 times, the amount calculated to form the normal fluoride of the amphoteric metal in its lower valence, i. e.,  $SbF_3$ ,  $SnF_2$  and  $BiF_3$ , on the basis of the available fluorine present in the chromia-fluorine-alumina catalyst.

There appears to be nothing critical in the method of preparing the catalysts of the present invention. In general, any method of catalyst preparation known to the prior art can be utilized. For example, the catalysts may be prepared by adding chromic acid and hydrogen fluoride, in

predetermined amounts, to an alumina base, followed by washing, drying, comminution and calcination under conditions adapted to yield products which have relatively high surface areas.

5 Or, alumina pellets may be impregnated, initially, with an aqueous solution of ammonium fluoride followed by washing, drying and calcining, and, subsequently, with an aqueous solution of chromic acid also followed by washing, drying and calcining, the amounts of fluorine and of chromia in the final catalyst being controlled by using calculated amounts of ammonium fluoride and of chromic acid, based on the weight of alumina and just enough water, in each case, to be completely absorbed by the pellets. The order of impregnation may be reversed or can be combined in one impregnation step. Or, commercially available or previously prepared chromia-alumina catalysts, in bead or pellet form, such as those 10 described in application for Patent Serial Number 201,537, filed by Stover and Wilson on December 14, 1950, may be impregnated with an aqueous solution of ammonium fluoride, the amounts of fluorine in the final catalyst being controlled by 15 using calculated amounts of ammonium fluoride and just enough water to be substantially completely absorbed by the beads or pellets.

Antimony, tin or bismuth can be introduced into the initial chromia-alumina gel by incorporating the sodium salts of the acidic oxides, such as sodium antimonate, sodium stannate and sodium bismuthate, into the sodium aluminate solution. Or, since the sulfides of antimony and tin are alkali-soluble, the finished chromia-fluorine-alumina catalysts can be impregnated with an ammonium sulfide solution of the metal sulfides.

Whatever the method of preparation employed, the catalyst is dried and then calcined. By way of non-limiting examples, the drying may be effected at temperatures of from about 300° F. to about 900° F., and the calcination, at temperatures varying between about 900° F. and about 1200° F., for a period of time of about one hour to about 10 hours.

45 It will be apparent to those skilled in the art that numerous compounds, can be used as sources for the various components of the catalysts contemplated herein. Thus, for example, fluorine may be introduced as dry hydrogen fluoride, aqueous hydrofluoric acid or an aqueous solution of ammonium fluoride ( $NH_4F$  or  $NH_4F \cdot HF$ ). Aqueous solutions of chromic acid, ammonium bichromate or chromium acetate may be used as sources of chromia.

55 Any of the commercially available aluminas of high surface area, such as gel-type alumina or "activated alumina," consisting principally of gamma-alumina, may be used to prepare impregnated catalysts of the type contemplated herein.

60 Or, precipitated alumina may be prepared in accordance with any known procedure suitable for the production of high-surface area alumina utilizable as a catalyst support. Thus, for example, aluminum hydroxide may be initially precipitated using aqueous solutions of aluminum nitrate, aluminum sulfate or aluminum chloride and the hydroxides or carbonates of ammonium, sodium or potassium. Residual sodium or potassium ions may be reduced to negligible amounts 65 by base-exchange with ammonium salts. Traces of residual sulfate, nitrate or chloride ions are not harmful.

Precipitation using a slight excess of alkali at a pH not exceeding 10 or using dilute solutions, 70 of the order of 0.1 molar or less, simplifies or fa-

cilitates the washing out of anions. Freezing and thawing the gelatinous, hydrous alumina converts it to a more easily filterable or centrifugable material and lowers its water-content, thereby facilitating washing. The addition of ammonium hydroxide or of neutral salts, such as ammonium nitrate, to the wash water facilitates the removal of other ions and prevents peptization of the alumina toward the end of the washing operation.

The method of addition of either the amphoteric metal or the fluorine is not critical but is limited by the solubilities of the compounds involved. The preparations given in the examples set forth hereinafter were selected to provide uniformity in the method of preparation rather than simplicity or economy. It will be apparent to those skilled in the art that various possible methods include:

(a) *Addition to gel-forming solutions*.—Any such additions should be made to the sodium aluminate rather than to the chromium acetate. The normal halides cannot be added because aluminum fluoride will precipitate if a soluble fluoride is added. Actually, antimony fluoride,  $SbF_3$ , is soluble while stannous fluoride,  $SnF_2$ , and bismuth fluoride,  $BiF_3$ , are not. However, the alkali salts of antimony and tin, such as sodium antimonate and sodium stannate, can be added to the sodium aluminate. The analogous bismuth salt, viz., sodium bismuthate, is water-soluble but is a powerful oxidizing agent, hence, although it can be used, it is not particularly desirable.

(b) *Impregnation*.—Wet impregnation is generally preferred because of better uniformity of impregnation; but it is not essential. The beads, for example, can be impregnated with antimony fluoride,  $SbF_3$ , but this will limit the atomic ratio of  $Sb:F$  to 1:3 (or 1.0 times the ratio of the normal, lower-valence fluoride).

Impregnation of either wet or dry beads with antimony or tin is best carried out with ammonium sulfide solutions of the antimony sulfide ( $Sb_2S_3$ ) or tin sulfide ( $SnS$ ) because the solutions do not damage the bead structure or do not introduce undesirable impurities. Sodium sulfide or potassium sulfide solutions can be used but this will necessitate following the impregnation with acidification to precipitate the sulfide, followed by washing and base-exchanging to remove the alkali metal ions. Bismuth sulfide ( $Bi_2S_3$ ) cannot be introduced in this manner because it is not soluble in alkali sulfides.

The other common salts of antimony, tin and bismuth, such as the nitrates and chlorides, hydrolyze easily and are soluble only in strongly acid solutions. Such solutions cannot be added to the wet beads because the acid will partially dissolve the alumina or the chromia or both. However, such solutions can be and have been used to impregnate dry beads.

The fluoride ion can be added separately or at the same time as the aqueous solution of the amphoteric metal, since it will not form a precipitate with the alkaline sulfide solutions of antimony or tin sulfides and will not precipitate in the strongly acid solutions of any of these metals ( $Sb$ ,  $Sn$ ,  $Bi$ ).

Fluorine is strongly adsorbed by (or reacted with) the surface and hence, is not easily washed out. Therefore, it can be added either before or after the addition of the amphoteric metal.

The catalysts can be used in any of the conventional forms such as powder, pills, spheres,

extrudates or irregular fragments, all of a size suitable for the reaction system to be employed.

Any mixture of hydrocarbons suitable as a charge stock to a reforming operation can be employed in the process of this invention. As is well known, petroleum naphthas, particularly those having a boiling range of from about 125° F. to about 450° F. and a relatively low octane number rating, are the conventional charge stocks for reforming processes of the type contemplated herein. Accordingly, the charge stock may be an intermediate type naphtha, i. e., one containing an average distribution of hydrocarbon types (paraffins, olefins, naphthenes and aromatics) or one which is exceptionally high in paraffins, naphthenes or aromatics.

The temperatures to be used in the process of the present invention vary between about 900° F. and about 1050° F., preferably, between about 975° F. and about 1025° F. The total pressures vary between about 100 pounds per square inch gauge and about 750 pounds per square inch gauge, preferably, between about 400 pounds per square inch gauge and about 600 pounds per square inch gauge. The mole ratios of hydrogen to naphtha vary between about 1:1 and about 10:1, respectively, preferably, between about 3:1 and about 6:1, respectively. The liquid hourly space velocities vary between about 0.5 and about 5 and, preferably, between about 2 and about 4.

The process can be carried out by making use of any of the well known techniques for operating catalytic reforming reactions in the vapor phase effectively. The reaction zone can be a chamber of any suitable type useful in contact-catalytic operations, for example, a catalyst bed contained in a shell, or a shell in which the catalyst is disposed in a series of beds, through which the hydrocarbons are passed in either upward or downward flow. The hydrocarbon vapors are maintained in contact with the catalyst at a predetermined elevated temperature and for a predetermined period of time, as set forth hereinbefore, and the resulting reaction mixture is passed through a condensing zone into a receiving chamber. It will be understood that the hydrogen can be recycled to the process.

It will be apparent that the process can be operated as a batch or discontinuous process as by using a catalyst-bed-type reaction chamber in which the catalytic and regeneration operations alternate. With a series of such reaction chambers, it will be seen that as the catalytic operation is taking place in one or more of the reaction chambers, regeneration of the catalyst will be taking place in one or more of the other reaction chambers. Correspondingly, the process may be continuous when one or more catalyst chambers through which the catalyst flows in contact with the hydrocarbon vapors is used. In such a continuous process, the catalyst will flow through the reaction zone in contact with the hydrocarbon vapors and will thereafter be separated from the hydrocarbon vapors as, for example, by accumulating the catalyst on a suitable filter medium, before condensing the reaction mixture. In a continuous process, therefore, the catalyst, fresh or regenerated, and the hydrocarbon vapors, fresh or recycled, will flow continuously through a reaction chamber.

The following detailed examples are for the purpose of illustrating the catalysts contemplated herein and to indicate the advantages and characteristics thereof, and, also, for the purpose of showing modes of carrying out the process of this

invention. It must be appreciated, however, that the invention is not to be construed as being limited to the specific catalysts, methods of catalyst preparation, and charge stocks disclosed herein-after or to the specific manipulations and conditions set forth in the examples. As those skilled in the art will readily understand, numerous modifications and variations therein, all within the purview of the foregoing discussion, are possible and, accordingly, must be considered to be encompassed by the scope of the present invention.

#### EXAMPLES 1-11

All the catalysts were prepared using chromia-alumina beads obtained in accordance with the procedure disclosed in application for patent Serial No. 201,537, filed by Stover and Wilson on December 14, 1950, referred to hereinbefore. Briefly, the procedure comprises rapidly mixing a solution of sodium aluminate (containing the equivalent of 2.65 moles  $\text{Al}_2\text{O}_3$  per liter) with a solution of chromic acetate (containing the equivalent of 0.75 mole  $\text{Cr}_2\text{O}_3$  per liter) in a mixing nozzle to form a chromia-alumina hydrosol. The hydrosol flows over a divider to form droplets and these fall through a column of oil. During the descent through the column of oil, the hydrosol droplets assume a spherical shape before setting to a firm hydrogel, thereby producing spherical hydrogel beads. The beads are then aged in an aqueous solution of ammonium sulfate, washed free of anions, dried in steam and, finally, calcined at a temperature of 1000° F. These beads approximate the composition:



The catalysts were prepared by treatment of dry, calcined beads with aqueous solutions containing the calculated amounts of desired component, assuming complete absorption, in just enough water to be completely absorbed.

In all cases, 0.03 gram atom of the metal per mole of chromia-alumina (one mole chromia-

amphoteric metals which obviated problems of hydrolysis and introduction of anions not decomposed by oxidation was impregnation with an acidic solution of the metal salt, precipitation of the metal as sulfide by re-impregnation with ammonium sulfide, followed by washing, drying and calcination in air for 3 hours at 950° F. to convert the sulfide to the oxide. The salts of the amphoteric metals used were stannous chloride acidified with hydrochloric acid to form a clear solution, antimony trichloride and bismuth nitrate acidified with nitric acid solution to give a clear solution.

One half of each of the chromia-alumina preparations containing 0.03 gram atom of the amphoteric metal oxide per mole of chromia-alumina was further impregnated with 0.06 gram atom of fluorine per mole of chromia-alumina by soaking the beads in just enough solution to be absorbed completely, the solution containing the calculated amount of ammonium fluoride to add the required amount of fluorine.

The wet beads were then dried overnight at temperatures of 176-212° F. in an air-circulation drying oven and then heated, in a hydrogen stream, at gradually increasing temperatures up to 950° F. over a 4-hour period and, finally, calcined for 3 hours in the hydrogen stream.

Catalyst evaluation was effected in conventional, stainless steel isothermal reactors, at temperatures of 1000° F., at liquid hourly space velocities of 1. The charge stock used was a light Oklahoma City naphtha having the following properties:

|                           |                       |            |
|---------------------------|-----------------------|------------|
| 35                        | Initial boiling point | 158° F.    |
| 10%                       | -----                 | at 175° F. |
| 50%                       | -----                 | at 190° F. |
| 90%                       | -----                 | at 212° F. |
| End point                 | -----                 | 248° F.    |
| CFRR octane number, clear | -----                 | 58.5       |

For convenience, the pertinent data are set forth in the following table:

Table

#### AVERAGE OF TWO ONE-HOUR TESTS WITH REGENERATED CATALYSTS

| Example No. | Catalyst,<br>$\text{Cr}_2\text{O}_3 : \text{Al}_2\text{O}_3 = 24 : 76$ | Atmospheric Pressure |                      |                                                      |                                 | 200 pounds per square inch gauge,<br>Mole Ratio = $\text{H}_2 : \text{Naphtha} :: 5:1$ |                      |                                                      |                                 |
|-------------|------------------------------------------------------------------------|----------------------|----------------------|------------------------------------------------------|---------------------------------|----------------------------------------------------------------------------------------|----------------------|------------------------------------------------------|---------------------------------|
|             |                                                                        | Gas, Wt.<br>Percent  | Coke, Wt.<br>Percent | C <sub>4</sub> -Free<br>Gasoline,<br>Vol.<br>Percent | CFRR<br>Octane<br>No.,<br>Clear | Gas, Wt.<br>Percent                                                                    | Coke, Wt.<br>Percent | C <sub>4</sub> -Free<br>Gasoline,<br>Vol.<br>Percent | CFRR<br>Octane<br>No.,<br>Clear |
| 1           |                                                                        | 17.6                 | 10.9                 | 69.0                                                 | 87.0                            | 19.4                                                                                   | 0.1                  | 78.5                                                 | 81.5                            |
| 2           | 0.03 K                                                                 | 14.2                 | 9.6                  | 73.5                                                 | 89.0                            | 18.5                                                                                   | <0.1                 | 80.5                                                 | 76.5                            |
| 3           | 0.03 K                                                                 |                      |                      |                                                      |                                 |                                                                                        |                      |                                                      |                                 |
| 3           | +<br>0.06 F                                                            | 12.8                 | 9.6                  | 73.0                                                 | 89.5                            | 16.2                                                                                   | <0.1                 | 82.5                                                 | 75.0                            |
| 4           | 0.03 Ca                                                                | 15.1                 | 11.1                 | 70.0                                                 | 90.5                            | 13.4                                                                                   | <0.1                 | 85.0                                                 | 75.5                            |
| 5           | 0.03 Ca                                                                |                      |                      |                                                      |                                 |                                                                                        |                      |                                                      |                                 |
| 5           | +<br>0.06 F                                                            | 12.3                 | 9.6                  | 74.5                                                 | 85.5                            | 17.5                                                                                   | 0.2                  | 81.0                                                 | 78.5                            |
| 6           | 0.03 Sp                                                                | 14.8                 | 10.2                 | 70.5                                                 | 92.5                            | 17.2                                                                                   | 0.1                  | 81.0                                                 | 78.0                            |
| 6           | 0.03 Sb                                                                |                      |                      |                                                      |                                 |                                                                                        |                      |                                                      |                                 |
| 7           | 0.03 Sb                                                                | 12.5                 | 9.5                  | 75.0                                                 | 81.5                            | 24.5                                                                                   | 0.5                  | 74.0                                                 | 88.5                            |
| 7           | +<br>0.06 F                                                            |                      |                      |                                                      |                                 |                                                                                        |                      |                                                      |                                 |
| 8           | 0.03 Sn                                                                | 12.4                 | 8.2                  | 75.5                                                 | 84.0                            | 16.0                                                                                   | <0.1                 | 83.0                                                 | 77.5                            |
| 8           | 0.03 Sn                                                                |                      |                      |                                                      |                                 |                                                                                        |                      |                                                      |                                 |
| 9           | +<br>0.06 F                                                            | 13.4                 | 10.2                 | 74.0                                                 | 82.5                            | 20.7                                                                                   | 0.1                  | 78.0                                                 | 83.5                            |
| 10          | 0.03 Bi                                                                | 14.4                 | 11.7                 | 70.0                                                 | 88.5                            | 22.3                                                                                   | 0.1                  | 75.5                                                 | 82.0                            |
| 10          | 0.03 Bi                                                                |                      |                      |                                                      |                                 |                                                                                        |                      |                                                      |                                 |
| 11          | +<br>0.06 F                                                            | 15.7                 | 10.9                 | 70.0                                                 | 78.0                            | 42.5                                                                                   | 0.7                  | 55                                                   | 91.5                            |

alumina is 0.24 mole  $\text{Cr}_2\text{O}_3$  plus 0.76 mole  $\text{Al}_2\text{O}_3$  ( $\text{Cr}_2\text{O}_3 : \text{Al}_2\text{O}_3 = 24 : 76$ ) was used. For potassium and calcium, the metal nitrates were used because they decompose on ignition to form metal oxides. A uniform technique for introducing the

75 The results set forth in the table show that all the metals, including potassium, calcium and the amphoteric metals, show a marked promoter action in the low-pressure runs. However, when the same catalysts were evaluated under hydro-

## 11

gen pressure, the promoter action became a depressor action. On the other hand, the catalysts containing both an amphoteric metal and fluorine, in accordance with the present invention, although showing a decreased activity at atmospheric pressure, showed a marked increase in activity under hydrogen pressure. The activity of the bismuth-containing chromia-fluorine-alumina catalysts was so great that the test conditions were entirely too severe for the catalyst. 10

What is claimed is:

1. A catalyst which comprises from about 5 per cent by weight to about 70 per cent by weight of chromium oxide, calculated as chromium sesquioxide, from about 0.1 per cent by weight to 15 about 2.0 per cent by weight of fluorine, an amphoteric metal selected from the group consisting of tin, antimony and bismuth, in amounts varying from about 0.5 to about 2 times the amount calculated to form the normal fluoride of the amphoteric metal in its lower valence, and the balance alumina. 20

2. A catalyst which comprises from about 10 per cent by weight to about 35 per cent by weight of chromium oxide, calculated as chromium sesquioxide, from about 0.2 per cent by weight to about 1.5 per cent by weight of fluorine, an amphoteric metal selected from the group consisting of tin, antimony and bismuth, in amounts varying from about 0.5 to about 0.75 times the amount calculated to form the normal fluoride of the amphoteric metal in its lower valence, and the balance alumina. 25

3. A process for effecting reforming of petroleum naphthas, which comprises contacting a petroleum naphtha with a catalyst comprising from about 5 per cent by weight to about 70 per cent by weight of chromium oxide calculated as chromium sesquioxide, from about 0.1 per cent by weight to about 2.0 per cent by weight of fluorine, an amphoteric metal selected from the group consisting of tin, antimony and bismuth, in amounts varying from about 0.5 to about 2 times the amount calculated to form the normal 30

5

20

25

30

35

40

## 12

fluoride of the amphoteric metal in its lower valence, and the balance alumina, at a temperature falling within the range varying between about 900° F. and about 1050° F., at a pressure falling within the range varying between about 100 pounds per square inch gauge and about 750 pounds per square inch gauge, at liquid hourly space velocities varying between about 0.5 and about 5, and in the presence of hydrogen in amounts varying between about one mole of hydrogen per mole of naphtha and about ten moles of hydrogen per mole of naphtha. 10

4. A process for effecting reforming of petroleum naphthas, which comprises contacting a petroleum naphtha with a catalyst comprising from about 10 per cent by weight to about 35 per cent by weight of chromium oxide, calculated as chromium sesquioxide, from about 0.2 per cent by weight to about 1.5 per cent by weight of fluorine, an amphoteric metal selected from the group consisting of tin, antimony and bismuth, in amounts varying from about 0.5 to about 0.75 times the amount calculated to form the normal fluoride of the amphoteric metal in its lower valence, and the balance alumina, at a temperature falling within the range varying between about 975° F. and about 1025° F., at a pressure falling within the range varying between about 400 pounds per square inch gauge and about 600 pounds per square inch gauge, at liquid hourly space velocities varying between about 2 and about 4, and in the presence of hydrogen in amounts varying between about 3 moles of hydrogen per mole of naphtha and about 6 moles of hydrogen per mole of naphtha. 20

WILLIAM H. LANG.  
CARLOS L. GUTZEIT.

## References Cited in the file of this patent

## UNITED STATES PATENTS

| Number    | Name   | Date           |
|-----------|--------|----------------|
| 2,427,800 | Mattox | Sept. 23, 1947 |